

Jan. 27, 1942.

M. SCHLÖTTER

2,271,209

ELECTRODEPOSITED TIN AND PROCESS OF ELECTRODEPOSITION

Filed Oct. 28, 1937

*Fig. 1.*



INVENTOR.

*MAX SCHLÖTTER.*

BY

*Beny. T. Rauher*  
ATTORNEY

## UNITED STATES PATENT OFFICE

2,271,209

ELECTRODEPOSITED TIN AND PROCESS OF  
ELECTRODEPOSITION

Max Schlötter, Berlin, Germany, assignor, by  
mesne assignments, of one-half to United  
States Steel Corporation, New York, N. Y., a  
corporation of New Jersey, and one-half to  
Carnegie-Illinois Steel Corporation, Pittsburgh,  
Pa., a corporation of New Jersey

Application October 28, 1937, Serial No. 171,420  
In Germany June 5, 1934

5 Claims. (Cl. 204—54)

This application is a continuation in part of  
my pending application Serial No. 25,000 filed  
June 5, 1935.

My invention relates to the electrolytic de-  
position of metals, particularly tin, in bright,  
glossy deposits.

Heretofore acid solutions of metal salts free  
from alkali and ammonium have been proposed  
for the electrodeposition of metals, such as tin,  
and the addition of colloidal substances or sub-  
stances in colloidal condition to the metal bath  
has been suggested. None of these suggested  
or proposed processes has, however, led to or re-  
sulted in the production of bright deposits di-  
rectly, but only to products which are coarsely  
granular or have a cloudy or clouded appearance.

My present invention provides an electrode-  
position of tin and other metals which is in such  
form as deposited as to give a bright and glossy  
appearance and provides, furthermore, a process  
whereby bright and glossy deposits of tin and  
other metals suitable for electroplating may be  
produced by electrolysis of acid metal baths.

In my present invention electrolysis of a solu-  
tion of a metal salt, for instance a tin salt, pre-  
ferably a stannous salt, in an acid containing  
aqueous medium is carried on under a greatly  
increased hydrogen over-voltage in the presence  
of a mixture of colloids, or of materials in col-  
loidal solution or state in said aqueous medium,  
at least one of the colloids being lyophilic or hy-  
drophile, or electro-negative, and at least one  
being a lyophobe or hydrophobe, or electro-posit-  
ive, to the solution and in which the electro-  
negative colloidal dispersed material is adsorbed  
or otherwise associated with the electropositive  
material, so that both migrate to the cathode.  
Otherwise expressed, one of the materials in  
colloidal dispersion in the acid tin or other metal  
bath would normally migrate to the anode, and  
the other one would normally or, if alone in the  
acid metal bath, migrate to the cathode. But  
when these two colloidally dispersed materials  
are both present in the electrolytic bath of my  
invention, they migrate to the cathode by elec-  
tro-osmosis, thus indicating that both of the  
colloids are associated in a larger dispersed par-  
ticle containing both electro-negative and elec-  
tro-positive dispersed particles, and having a  
residual positive charge. Some of the metal ions  
may also be adsorbed in this larger colloidal ag-  
gregate of positive and negative or hydrophobe  
and hydrophile particles. It will be understood  
that these colloids may be present in very small

amounts. Preferably, they are of organic non-  
conducting materials or substances.

The combination of colloids thus obtained in  
my electrolytic bath has the effect of greatly  
increasing the hydrogen over-voltage over that  
which could be obtained by using either of the  
colloidally dispersed materials alone, even in an  
amount equal to the total of both colloids. This  
increase in over-voltage permits the production  
of an electro-deposition of novel structure that is  
highly advantageous.

In the accompanying drawing the figure is  
a graph showing the relation between over-  
voltage in milli-volts as abscissae and corre-  
sponding current densities as ordinates for tin  
baths of identical composition except that some  
contain resins in different proportions, others  
gelatin and others a mixture of gelatin and  
resin.

As shown in the drawing, for example, 0.4%  
of resin increases the over-voltage somewhat.  
The presence of 0.2% of resin and 0.2% of gela-  
tin increases the over-voltage much more, par-  
ticularly at the lower current densities. The in-  
crease over the over-voltage obtained with gel-  
atin alone is even greater.

In the electrolysis of acid tin baths according  
to my invention, therefore, to an acidified aque-  
ous stannous solution, there are added at least  
two different colloids, one being a hydrophobic  
colloid electro-positive to the solution, and the  
other a hydrophilic colloid electro-negative to  
the solution, the two colloids being organic ma-  
terials and not mutually precipitated, nor pre-  
cipitated by the tin or acid of the solution, so  
as to form a substantially permanent colloidal  
solution. The two opposite colloidal materials  
are so chosen that the negatively charged par-  
ticles will be adsorbed to, or will aggregate with,  
the positively charged materials so that both  
will migrate to the cathode.

Electrolysis is then carried on through this  
bath by the passage of current from a tin anode  
to the material to be plated at the cathode. The  
current density will be sufficient to provide a  
high hydrogen over-voltage. This current den-  
sity is about at the point, or slightly above the  
point, at which hydrogen is discharged at the  
cathode. In other words, the current density  
in each case is increased until minute bubbles  
of hydrogen appear.

A large number of substances may be em-  
ployed in conjunction to form a hydrophilic, or  
positively charged, and a hydrophobic, or nega-  
tively charged, dispersion. Examples of hydro-

phile or lyophile colloids are glue, gelatin, agar-agar and albuminous substances. Examples of hydrophobe or lyophile colloids are bitumen, cellulose derivatives, sulphonated oils, tars, for instance, wood tar such as beechwood tar or birchwood tar, and the like. Phenolic or cresylic resins, that is, synthetic resins obtained as condensation products of phenol, or cresol, are particularly advantageous for use as hydrophobe colloids in combination with hydrophile colloids. Examples of such colloid combinations are as follows:

Glue and beechwood tar  
 Gelatin and bitumen  
 Agar-agar and cellulose derivatives  
 15 Glue and phenol or cresol resin  
 Gelatin and beechwood tar  
 Glue and extract from sulphite lignose with sulfonic acids

By electrical charge is meant the charge of the particle in the particular electrolytic bath solution although it may have a different charge in another medium, an alkaline one, for example. An instance is the dispersed rubber of latex, which is negative when the dispersing medium is alkaline and positive when the dispersing medium is acid. Also the composite dispersed particles will have a residual positive charge and move to the cathode where they will cause a greatly increased hydrogen overvoltage as compared with either of the charged particles alone. It will be also understood that the term phenol includes all aromatic compounds having the phenol radical and that glue includes gelatin, albuminous substances, agar agar and similar gelatinous materials.

It will be understood that the above combinations are given merely by way of example and that the various colloids may be arranged in different combinations. Certain organic compounds, for example, certain dyestuffs such as benzo-purpurin, or Congo red, or similar long compounds of high molecular weight form molecules coming within the molecular size range, that is, between 1 milli-micron ( $\mu\mu$ ) to about 0.5 micron ( $1\mu$ ), or more than one-millionth to one-thousandth of a millimeter in dimension, may therefore be used as colloids in my process in conjunction with a colloidal dispersion of opposite charge.

The materials of opposite charge may be dispersed to colloidal condition in any suitable manner as is well known in the art.

Solvents that are miscible with water may be added to aid in the distribution or dispersion of the colloids, especially the resins therein, and to assist their dispersion at the cathode. For example, a mixture of 10% acetone in alcohol may be added to the bath. Other solvents, such as dioxan, may be added or used in the dispersion of the material. These added solvents serve to stabilize, or to increase the stability, of the colloidally dispersed material, and are necessary or advantageous only with certain dispersions. The solvent will be selected with a view to the nature of the dispersion. For example, in a dispersion of wood tar, the acetone may be omitted.

In the electro-deposition of metals which 70 commonly have more than one valence as, for example, in the case of tin which occurs as bivalent or stannous and quadrivalent or stannic salts, the electrolysis should be from a solution containing substantially only the stannous ions. 75

Electro-deposition from a stannic solution forms a coarser, more roughly crystalline deposit, while electro-deposition from a solution containing a mixture of stannic and stannous ions generally results in a more spongy deposition. To obtain dense, finely grained and lustrous or glossy deposits of tin, electrolysis should therefore take place from a solution which contains a small or negligible quantity, or no, stannic ions and should be under such conditions as to avoid or prevent the formation of stannic ions.

The formation of stannic ions in the electrolytic bath may be avoided or prevented by using tin salts of organic sulphonates and avoiding 15 the tin salts of the usual inorganic or mineral acids. The aromatic sulphonates are the ones useful for this purpose, as they have a much greater stability under the conditions of electrolysis than do the aliphatic sulphonates or 20 sulphonates of straight chain compounds. For example, the mono- or polysulphonates of such ring compounds as benzene, toluene, xylol, phenol, cresol, mono- or polysulphonates, the disulphonates of naphthalene, and even sulphonates of multiple ring compounds, such as 25 anthracene, may be employed.

In making a solution of the tin salt of sulphonic acid, a tin sulphonate may be dissolved to the required concentration or, a solution of 30 sulphonic acid may be added to a solution of a tin sulphate and, if the concentration of inorganic acid is too high, it may be lowered by the addition of a barium sulphonate or other suitable barium compound or, a suitable tin 35 sulphonate may be obtained by admixing solutions of a stannous sulphate and barium sulphonate in proper proportions. The resulting barium sulphate may be separated by filtration or decantation, etc. Or, tin may be dissolved directly in a suitable aromatic sulphonic acid.

In making up a bath for electroplating tin, therefore, an organic sulphonate is commonly used. An example of such a sulphonate would be an aromatic sulphonate of tin, such as tin 40 cresol sulphonate or tin phenol sulphonate, which are common aromatic sulphonates. The concentration of the tin salts may vary. Concentrations of less than 10% (for example, about 4-5% of tin as cresol sulphonate or phenol sulphonate) are generally employed. Such a solution will also contain the positively and negatively charged colloids as, for example, dispersed phenolic resins and glue; for example, as colloidal aggregates. Electrolysis conducted at a 45 density of from 2 to 6 amperes per square decimeter will give a bright or lustrous, fine grained, adherent, deposit of tin.

For other metals, analogous means may be employed in the preparation of suitable electrolytes.

It will be understood that, although the presence of inorganic anions or inorganic acids or salts is undesirable from the standpoint of producing deposits of high gloss, a small amount as, for example, 4% or 5% of stannous sulphate may not be objectionable.

It will be understood also that any suitable means for colloidally dispersing the dispersed materials may be employed. In the case of glues, gelatins, etc., the dispersion takes place readily by merely soaking the material in water. In the case of resins, tars, etc., dispersion may take place by means of a common solvent in which the resin or tar may be dissolved and then poured into the water with vigorous stirring.

Other methods that have heretofore been employed for colloidally dispersing materials in an aqueous medium as, for example, electrolytic methods, formation of insoluble materials in situ in minute dispersion in the dispersing medium as, for example, forming the resin from resin-forming ingredients and diluting, etc., may be employed. These methods are, however, merely examples of the various methods of colloidally dispersing materials. The presence of the colloidally dispersed materials of opposite charge in the acidic electroplating bath is evidenced by an increased hydrogen overvoltage over that obtained by one of the colloids alone, particularly at low current densities. This is apparent from Fig. 1 of the drawing.

Representative examples of electrolytic baths using my invention are as follows:

*Example I*

|                                  |      |      |
|----------------------------------|------|------|
| Tin in the form of stannous salt | gms. | 25   |
| Sulphuric acid of 66° Baumé      | gms. | 75   |
| Glue                             | gm.  | 1    |
| Phenol resin                     | gms. | 1.5  |
| Alpha-naphthol                   | gm.  | 0.5  |
| Water                            | cc.  | 1000 |

*Example II*

|                                             |      |      |
|---------------------------------------------|------|------|
| Tin in the form of tin benzene disulphonate | gms. | 30   |
| Benzene disulphonic acid                    | gms. | 90   |
| Gelatin                                     | gm.  | 0.8  |
| Beech wood tar                              | cc.  | 0.5  |
| Water                                       | cc.  | 1000 |

*Example III*

|                             |      |      |
|-----------------------------|------|------|
| Sn as stannous salt         | gms. | 25   |
| Naphthalenedisulphonic acid | gms. | 115  |
| Glue                        | gm.  | 1    |
| Benzoin resin               | gm.  | 0.8  |
| Alcohol                     | cc.  | 3    |
| Water                       | cc.  | 1000 |

*Example IV*

|                            |      |       |
|----------------------------|------|-------|
| Benzoldisulphonate of zinc | gms. | 220   |
| Glue                       | gm.  | 0.5   |
| Licorice root extract      | cc.  | 10-20 |
| Beechwood tar              | cc.  | 1     |
| Water                      | cc.  | 1000  |
| pH                         |      | 2-5   |

*Example V*

|                     |      |      |
|---------------------|------|------|
| Cadmium perchlorate | gms. | 250  |
| Agar-agar           | gm.  | 0.5  |
| Benzo-purpurine     | gm.  | 1    |
| Water               | cc.  | 1000 |
| pH                  |      | 2-5  |

*Example VI*

|                         |      |      |
|-------------------------|------|------|
| Copper phenolsulphonate | gms. | 200  |
| Copper perchlorate      | gms. | 50   |
| Perchloric acid         | gms. | 40   |
| Latex                   | gm.  | 0.05 |
| Acetone                 | gms. | 1.5  |
| Gelatine                | gm.  | 0.1  |
| Water                   | cc.  | 1000 |

*Example VII*

|                           |      |      |
|---------------------------|------|------|
| Lead perchlorate          | gms. | 250  |
| Cresylsulphonic acid      | gms. | 80   |
| Extract of caragheen moss | cc.  | 10   |
| Beechwood tar             | gm.  | 1    |
| Water                     | cc.  | 1000 |

In electrolysing the above baths, metal deposits are obtained using a current density of

from about 3 to 6 amperes per square decimeter in a still bath. In an agitated bath very much higher current densities may be employed. These deposits have a fine grain which cannot be detected under the finest microscope and must, therefore, be below the wave length of light, that is less than 0.4 micron ( $\mu$ ).

Not only are the crystals of which the electro-deposit is formed of very small size or dimension, but their internal structure is modified by the introduction in the crystal lattice or unit of a metal compound. In the deposit obtained by my invention, however, one or more of these atoms are replaced by anion-like bodies, for instance, sub-oxides, hydroxides, oxides, etc., of the metal. This replacement of an atom of the metal by a molecule of one of its compounds, or of several atoms by the same number of said molecules, causes an enlargement of the crystal lattice and, therefore, a change in the axial ratio. If, for instance, the axial ratio before introduction of said molecule or molecules was  $a:b:c$ , now one of the axes has become elongated and the ratio is now  $a:b:(c+\alpha)$ . Through this change new physical and chemical properties are imparted to the metal as, for instance, high gloss. Each of the crystals thus formed will have dimensions less than the wave length of light, that is, less than about 0.4 micron. These crystals are not only of small size, but they have what is known as a "preferred orientation," that is, they are all orientated in the same direction. As distinguished from random orientation, crystals orientated in the same direction have an axis of each crystal in substantial parallelism or alignment with corresponding axes of the other crystals and this brings corresponding faces of the crystals into parallelism. For example, X-ray examination of plane sheet products of this invention have shown corresponding axes of each of the crystals to be at substantially a right angle to the surface of the deposit. These various structures are not detectable by the use of a microscope and the ordinary light rays, but may be determined by the use of X-rays which have a much smaller wave length than the ordinary light rays.

The deposit may also be recognized by a visual inspection because of its very high gloss and because its crystal structure is not detectable with a microscope. In contradistinction to formerly known deposits, the deposits of my invention have a uniform high gloss surface. Where the gloss is too high for commercial use, it may be reduced by brushing with brushes of soft wire, for example, brushes made of German silver wire, in order to reduce the gloss to any desired commercial standard.

Other addition agents besides the colloids may be added as, for example, agents which lower the surface tension of water, known commonly as capillary active substances, for example, lauric acid, certain amines and phenol, such as alpha-naphthol, given in Example I, or sulphonated oils as, for example, Turkey red oil. Such materials may be added either during the dispersion of the colloids, or afterwards.

What I claim is:

1. A process of electro-plating tin which comprises passing an electric current from a tin anode to a cathode to be electro-plated through an aqueous solution of an aromatic sulphonate of tin, said solution containing colloidally dispersed phenolic resins and glue in proportions to form electro-positive colloidal aggregates, and con-

ducting said electrolysis at a current density of from 2 to 6 amperes per square decimeter.

2. A process of electroplating tin which comprises passing a current from a tin anode to a cathode to be plated through an aqueous plating bath containing a solution of stannous salts, said salts being predominantly organic sulphonates of tin, an acid and colloidally dispersed aggregates electropositive to said solution said aggregates comprising a dispersed material of the group consisting of the phenolic and cresylic resins, bitumens, wood tars, extract from sulphite lignose with sulfonic acids, and cellulose derivatives, electro-positive to said solution and material electronegative to said solution adsorbed on said electropositively charged particles and maintaining a cathode current density upward of 2 amperes per square decimeter.

3. A process of electroplating tin which comprises passing an electroplating current from a tin anode to a cathode to be electroplated through an aqueous solution of an aromatic sulphonate of tin, said solution containing an acid, colloidally dispersed aggregates electro-positive

to said solution and comprising material of the group consisting of the phenolic and cresylic resins, bitumens, wood tars, extract from sulphite lignose with sulfonic acids, and cellulose derivatives, electropositive to said solution and material electronegative to said solution adsorbed on said electropositively charged material and comprising a member of the group consisting of glue, gelatin, agar-agar and albuminous materials, and maintaining a cathode current density upward of 2 amperes per square decimeter.

4. A base metal having a bright or glossy electrodeposit of tin the crystals of which have a size approximating the wave length of light and are all orientated in the same direction.

5. A bright or glossy electro-deposit of tin having a crystal size approximating the wave length of light, said deposit having a crystal lattice, said crystal lattice comprising tin atoms and a small quantity of a compound of the group consisting of tin hydroxide, tin oxide and tin suboxide and the crystals of said deposit being all orientated in the same direction.

MAX SCHLÖTTER.